

## UNITED STATES PATENT OFFICE

2,071,463

## FILM

Max Hagedorn and Armin Ossenbrunner, Dessau  
in Anhalt, and Gustav Wilmanns, Wolfen Kreis  
Bitterfeld, Germany, assignors to Agfa Ansco  
Corporation, Binghamton, N. Y., a corpora-  
tion of New York

No Drawing. Application March 2, 1934, Serial  
No. 713,771. In Germany March 4, 1933

4 Claims. (Cl. 106—40)

Our present invention relates to the manufacture of film.

One of its objects is to provide a process for the manufacture of film having improved mechanical properties. Another object is the improved film. Further objects will be seen from the detailed specification following hereafter.

According to this invention it has been found that compounds having no dissolving action on cellulose esters and which are derived from the paraffins and the high boiling carbon hydrates available in nature, are particularly suited as softening agents for organic cellulose esters and mixed organic and inorganic cellulose esters, for instance, cellulose acetate, cellulose nitroacetate, and cellulose acetobutyrate. The softening agents according to this invention are the esters of monovalent alcohols with fatty acids or the alcohols which are obtainable by oxidation of the above mentioned paraffins and high boiling hydrocarbons, such as are resulting in the hydrogenation under pressure of coal or brown coal, or in cracking the hydrocarbons contained in the high boiling fractions. In view of the heterogeneity of the starting material, the fatty acids or the alcohols are obtained in form of mixtures which may differ in accordance with different oxidizing processes. They contain nearly all arborescent carbon chains and therefore differ principally from the natural fatty acids or the alcohols obtainable from the fatty acids by reduction. If the esters shall be suitable for the manufacture of supports for photographic layers they must not contain strongly smelling compounds. For the purposes of the invention there are particularly suited the esters which are derived from fatty acids having an unbranched chain of at least 8 carbon atoms or the alcohols having an unbranched chain of at least 8 carbon atoms. The lower esters or alcohols are not so useful because they have a high vapor pressure and therefore are very volatile. The softening agents prepared by oxidizing paraffins such as lignite wax and ozocerite, or the high-boiling brown coal oils by means of air (with or without a catalyst), nitric acid or chromic acid are preferred without limiting the invention.

The following examples serve to illustrate the invention:

Example 1.—Acetylcellulose containing 56 per

cent. of acetic acid is dissolved in a mixture of methylene chloride, chloroform and amyl alcohol in the proportions of 2:5:2 to a solution of 18 per cent strength while adding 20 per cent of the alcohols obtained by oxidizing commercial paraffin. The solution obtained is cast to form a film of 0.135 mm. thickness. This film shows the following data in comparison with a film prepared with triphenylphosphate, the usual softener for acetylcellulose.

| Kind of addition                                                  | Breaking load, kilo | Elongation, percent | Creasing number |    |
|-------------------------------------------------------------------|---------------------|---------------------|-----------------|----|
| 20 per cent of alcohols obtained by oxidizing commercial paraffin | 88                  | 42                  | 335             | 15 |
| 20 per cent of triphenylphosphate                                 | 89                  | 37                  | 191             |    |

Example 2.—To a solution of 180 grams of cellulose acetobutyrate in 820 grams of a mixture of acetone and alcohol in the ratio 8:2 there are added 36 grams of the butylester of the mixture of fatty acids obtained from lignite wax by oxidation with chromium acid. From this mixture there is cast a film of 20 to 25  $\mu$  thickness which in view of its good mechanical properties as to elasticity, extensibility and creasing number is much better adapted for insulating electric conductors than film without the addition of softening agent or with the addition of triphenylphosphate or tricresylphosphate or phthalic acid esters hitherto used.

What we claim is:

1. A process of manufacturing film which comprises dissolving cellulose acetate containing 56 per cent of acetic acid in a mixture of methylene chloride, chloroform and alcohol, adding a mixture of alcohols obtained by oxidizing commercial paraffin and casting the film from this solution.

2. A film which comprises cellulose acetate containing 56 per cent of acetic acid and a mixture of alcohols obtained by oxidizing commercial paraffin.

3. Process of manufacturing film which comprises dissolving in a suitable solvent therefor a compound selected from the group consisting of organic acid esters of cellulose and mixed organic-inorganic acid esters of cellulose, adding

5

10

15

20

25

30

35

40

45

50

thereto a non-solvent mixture of alcohols obtained by oxidizing a hydrocarbon mixture selected from the group consisting of paraffin wax, lignite wax, ozocerite, and high-boiling hydrocarbons of the type of brown coal oils, most of said alcohols having an arborescent chain of carbon atoms, and casting the film from this solution.

4. A cast film comprising a compound selected from the group consisting of organic acid esters of cellulose and mixed organic-inorganic acid

esters of cellulose in admixture with a non-solvent mixture of alcohols obtained by oxidizing a hydrocarbon mixture selected from the group consisting of paraffin wax, lignite wax, ozocerite, and high boiling hydrocarbons of the type of brown coal oils, most of said alcohols having an arborescent chain of carbon atoms.

MAX HAGEDORN.

ARMIN OSSENBRUNNER.

GUSTAV WILMANNS.

10